

## UNITED STATES PATENT OFFICE

2,126,818

## GAS-RETAINING FABRIC

THERON P. SAGER AND DAVID F. HOUSTON,  
WASHINGTON, D. C.No Drawing. Application August 22, 1936,  
Serial No. 97,448

2 Claims. (Cl. 91—68)

(Granted under the act of March 3, 1883, as  
amended April 30, 1928; 370 O. G. 757)

This invention relates to the treatment of fabrics employed for the retention of lifting gases in lighter-than-air craft, and it particularly relates to the provision of a gas impermeable coating for such fabrics.

One object of the invention is to provide a coating material which may be readily applied by calendering, brushing, spraying, or spreading.

Another object is to provide a coating which shall be highly flexible and durable under varying conditions of atmospheric exposure.

It is customary in the construction of gas-retaining fabrics to apply a film or coating to the surface of the fabric which will prevent the diffusion of the enclosed gases. Rubberized fabric has been employed as a gas-retaining medium. Rubberized fabric is relatively inexpensive and easily manufactured, but a film of rubber is inherently permeable to gases and the use of rubberized fabric in the construction of gas cells results in a high loss of lifting gases. Varnishes, lacquers, and dopes having cellulose derivatives as their basic materials have been suggested as gas retaining films. Those which have been proposed have not, however, been wholly satisfactory, either because of their high rate of diffusion to gases or because they tend to crack on flexing of the coated fabric. Another class of materials which is employed as coatings for gas-retaining fabrics includes substances such as goldbeater's skin, gelatin, and regenerated cellulose. These materials, while highly impermeable to lifting gases, all have a fault in common in that they are maintained in a flexible condition by the presence of glycerol or similar hygroscopic plasticizer. The presence of a hygroscopic plasticizer causes a wide variation in the weight of the coated fabric under varying conditions of atmospheric humidity. A further objection to the use of these materials is that they are readily subject to attack by mold and bacteria.

This invention consists in the discovery that films containing an olefine-polysulphide reaction product are highly impermeable to hydrogen and helium, and in addition the foregoing disadvantages of gas-retaining fabrics formerly proposed may be overcome by employing as a coating on such fabrics an olefine-polysulphide reaction product. A fabric thus coated possesses the characteristic flexibility of rubber but differs from rubber in having a low permeability to lifting gases. The term olefine-polysulphide reaction product relates to a plastic material obtained by the interaction of alkaline or alkaline earth polysulphides and organic compounds containing

methylene or substituted methylene groups, and particularly to additive halogen derivatives of such compounds. Such a material may be applied to a fabric by any of the customarily employed methods. In the form of a plastic mass it may be calendered. Dispersed in a suitable solvent it may be sprayed, brushed, or spread with a spreading machine. The material may be employed as an impermeable coating unmixed with any other material and not subjected to any heat treatment. To obtain, however, the most satisfactory physical characteristics it has been found desirable to compound it with varying amounts of rubber, pigments, accelerators, and vulcanizing agents. Likewise, it has been found desirable to cure the coated fabric at elevated temperatures to obtain the most satisfactory strength and flexibility. A fabric coated with an olefine-polysulphide reaction product is remarkably resistant to water and organic solvents, notably the hydrocarbons. It has also been found to be highly impermeable to hydrogen and helium.

In the following examples illustrative of our invention the olefine-polysulphide reaction product referred to therein was of a grade known as "Thiokol B", prepared by the Thiokol Corporation, Yardville, New Jersey. The scope of this invention is not, however, limited to this particular grade of material.

## Example 1

One hundred grams of olefine-polysulphide reaction product was dissolved in 1000 grams of carbon disulphide and applied to a closely woven balloon fabric by brushing. The balloon fabric weighed 2 ounces per square yard. The coating was dried at 125° F. until all residual solvent was driven off. The coated fabric weighed 5.7 ounces per square yard and gave a diffusion rate of 0.5 liter per square meter per 24 hours.

## Example 2

A material serving as another example was composed as follows in parts by weight:

|                                       |     |
|---------------------------------------|-----|
| Olefine polysulphide reaction product | 100 |
| Zinc oxide                            | 10  |
| Tetramethylthiuram disulphide         | 0.2 |

The materials were mixed on a differential speed roll mill. The mixture was then dispersed in a solvent mixture containing 900 parts by weight of carbon disulphide and 100 parts of chlorbenzene to form a solution containing 10 per cent by weight of solid material. This solution was

then applied to a closely woven balloon fabric by brushing on a plurality of coats. The coated fabric was cured in a drum in open steam for 60 minutes at 264° F.

- 5 The cured fabric, which weighed 5.6 ounces per square yard, gave a diffusion rate of 0.4 liter per square meter per 24 hours.

*Example 3*

- 10 A mixture composed in parts by weight of the following was prepared:

|                                       |      |
|---------------------------------------|------|
| Olefine-polysulphide reaction product | 100  |
| Smoked sheet rubber                   | 10   |
| Zinc oxide                            | 10   |
| 15 Carbon black                       | 20   |
| Tetramethylthiuram disulphide         | 0.25 |

20 The rubber was incorporated with the olefine-polysulphide reaction product on a differential speed roll mill. The remaining ingredients were added and the whole was milled to a uniform plastic mass. The mixture was then dispersed in 1100 grams of beta trichlorethane. The resulting solution was spread on a closely woven balloon fabric, weighing 2 ounces per square yard, by means of a spreading machine. The coated fabric was cured in dry heat for 60 minutes at 264° F. The permeability of the cured fabric, which weighed 5.8 ounces per square yard was 30 1.7 liters per square meter per 24 hours.

*Example 4*

This example illustrates the adaptation of our invention to a variation of coated fabric construction. To a closely woven balloon fabric was applied the following in parts by weight:

|                               |      |
|-------------------------------|------|
| Smoked sheet rubber           | 100  |
| Zinc oxide                    | 10   |
| Stearic acid                  | 1    |
| 40 Sulphur                    | 0.6  |
| Tetramethylthiuram disulphide | 0.25 |
| Mercaptobenzothiazole         | 1    |
| Benzol                        | 3600 |

45 The solution was applied to the fabric with a spreading machine to the amount, upon evaporation of the solvent, of 0.6 ounce per square yard.

To the preponderantly rubberized surface of this fabric was then applied a material composed in parts by weight of the following:

|                                       |      |
|---------------------------------------|------|
| Olefine-polysulphide reaction product | 100  |
| Smoked sheet rubber                   | 50   |
| Zinc oxide                            | 10   |
| Tetramethylthiuram disulphide         | 0.25 |
| 55 Beta trichlorethane                | 1800 |

55 The solution was applied with a spreading machine. The amount of coating applied was 0.8 ounce per square yard.

To this coated surface was then applied the following mixture in parts by weight:

|                                       |      |
|---------------------------------------|------|
| Olefine-polysulphide reaction product | 100  |
| Zinc oxide                            | 10   |
| Tetramethylthiuram disulphide         | 0.1  |
| 65 Beta trichlorethane                | 1100 |

The amount of coating deposited from this mix-

ture was 2.6 ounces per square yard. The coated fabric was then heated in dry heat for 60 minutes at 264° F. In this method of construction the intermediate coating serves as an adhesive layer by which the outer coating of olefine-polysulphide reaction product is attached to the rubberized fabric.

In the foregoing examples the functions of the various compounding ingredients are as follows:

Rubber is added to improve the tensile strength 10 of the compounded material. Zinc oxide is an important ingredient which materially assists in altering the properties of the olefine-polysulphide reaction product during the final heat treatment 15 with the result that the material is rendered more resilient and resistant to abrasive action. Carbon black increases the toughness of the mixture. Tetramethylthiuram disulphide, mercaptobenzothiazole, sulphur and stearic acid improve the 20 properties of the compounded material by assisting the curing of the rubber and the olefine-polysulphide reaction product.

The foregoing examples are given merely for purposes of illustration. Numerous modifications 25 are possible and will be apparent.

Other modifications and changes in the proportions and arrangements of the parts may be made by those skilled in the art without departing from the nature and scope of the invention, as defined in the appended claims.

The invention described herein may be manufactured and used by or for the Government of the United States of America for governmental purposes without the payment of any royalties 35 thereon or therefor.

Having thus set forth and disclosed the nature of this invention, what we claim is:

1. The method of providing a balloon fabric impermeable to lifting gases which comprises applying a gas impervious continuous film to a closely woven balloon fabric weighing approximately two ounces per square yard, the fabric being first rubberized before the continuous film is applied, the continuous film including a coating composition comprising an olefine-polysulphide 45 reaction product and rubber, the olefine-polysulphide reaction product being the basic ingredient of the composition and providing the impermeability factor to the fabric, whereby the completed impermeable balloon fabric has its weight 50 increased from two and four-fifths to three times its original weight.

2. A balloon fabric impermeable to lifting gases comprising a closely woven fabric weighing approximately two ounces per square yard, a rubberized coating on said fabric and a continuous gas impervious film on said rubberized fabric, said film comprising an olefine-polysulphide reaction product and rubber, the olefine-polysulphide product being the basic ingredient of the composition and providing the impermeability factor to the completed fabric, the completed fabric 60 weighing from two and four-fifths to three times the weight of the original fabric.

THERON P. SAGER. 65  
DAVID F. HOUSTON.